

## UNITED STATES PATENT OFFICE

GUSTAV KOMAREK, OF CHICAGO, ILLINOIS, ASSIGNOR TO BERMUND FUEL COMPANY OF DELAWARE, OF CHICAGO, ILLINOIS, A CORPORATION OF DELAWARE

## BRIQUETTE AND PROCESS FOR MAKING SAME

No Drawing.

Application filed June 20, 1929. Serial No. 372,545.

The present invention relates to fuel briquettes, and has as an object to provide a briquette of improved composition and a new and improved process for the manufacture of briquettes.

An object of the invention is to reduce the formation of dust in the manufacture and handling of the briquettes, and also to improve the briquette for combustion purposes, more particularly by reducing the smoke given off during combustion.

Briquettes are ordinarily made from finely divided carbonaceous material, such as anthracite or bituminous coal, coke fines, or petroleum coke, and an improved briquette composition involving the use of petroleum coke and other material of low volatile content, such as coke fines, is disclosed in my Patent 1,796,465, Mar. 17, 1931.

Briquettes of these compositions have one fault in common with coal or coke, namely, the dust which is produced by the abrasion set up in handling. Briquette dust is particularly objectionable, due to the loss of combustible material, and furthermore, because of the binder which makes the dust sticky, and, therefore, more objectionable than dust of ordinary coal or coke.

It is, of course, old and well known to utilize various chemicals for allaying coal dust, and their use is extensively treated in Bulletin 20 of the Bureau of Mines, (Government Printing Office, 1911) entitled "The Explosibility of Coal Dust". However, so far as I am aware, the use of deliquescent materials has heretofore never been extended to briquettes. Their use in briquette manufacture is attended with problems, such as the deterioration of the briquette by the chemicals, which is more serious than any deterioration due to dust formation.

Briquettes ordinarily comprise the combustible mass, such as coal, coke, or a combination of these, and a binder. Binders are of two general classes, namely, (1) those impervious to moisture, such as coal tar pitch and asphalt, and (2) those susceptible to moisture and somewhat hygroscopic, such as sulphite liquor and starch.

When either class of binder is used it has

heretofore been customary to dry out and heat the combustible mass of coal, since the presence of any material amount of moisture in the coal will seriously impair the adhesive effect of the binder. Consequently, old and well known processes heretofore employed for allaying coal dust are not practicable, since the heating and drying of the coal to remove moisture, would at the same time remove the hygroscopic material applied to the coal.

Furthermore, the inclusion of a deliquescent material in the briquette would, naturally, be regarded as objectionable, for the reason that its hygroscopic action would deteriorate the binder, and, by impairing the adhesive qualities of the latter, break down the briquette. For these reasons any hygroscopically active material heretofore used in the briquettes have been employed for other than hygroscopic action and have been chemically neutralized, thus eliminating any tendency to absorb moisture.

I have discovered that it is possible, and desirable, to use in briquettes a deliquescent material, and particularly a deliquescent salt, such as calcium chloride ( $CaCl_2$ ), magnesium chloride ( $MgCl_2$ ), or a material such as potassium carbonate ( $K_2CO_3$ ). These materials by their hygroscopic action improve the briquette, and not only prevent the formation of dust, but also slow down combustion, thereby reducing the amount of smoke given off. This retardation of combustion renders necessary high temperatures before volatile gases contained in the binder or combustible material can evolve.

In the use of the deliquescent material, particular care must be exercised to see that it is free or available, as such, after the briquette has been manufactured, so as to be hygroscopically active. This phase of my invention involves in its application to briquette manufacture particular attention to the nature of the binder employed. If, in the briquette, a binder or other material is used, which tends to combine or react chemically with the deliquescent material, then a sufficient amount of such deliquescent material must be used over and above that part

which combines with or is neutralized by the binder or any other ingredient, in order that it may be free or available for hygroscopic action. This phase of the invention may also be carried out by employing a binder including other materials chemically inactive or substantially inert relative to the deliquescent salt; if this is done it is not necessary to take into consideration any chemical activity in determining the amount of deliquescent salt to be employed.

But whether the binder used be chemically active or inactive relative to the deliquescent salt, the latter should be used in such an amount, and applied in such a way, as to be free for hygroscopic action. Also it must be employed in the manufacturing process in such a way as not to break down the adhesion of the combustible particles produced by the binder. This may be accomplished by controlling the amount of deliquescent material used, and also by following my improved process, which involves varying the mode of including the deliquescent material or salt in the briquette.

In the manufacture of practically all briquettes the moisture is largely removed from the combustible mass of carbonaceous material before it is mixed with a binder. This mass consists of finely divided material, such as anthracite or bituminous coal. The carbonaceous material is then mixed with a suitable binder, and to this mixture the deliquescent material may be added in dry form, particularly when steam is introduced during the kneading or mixing operation. Such material as deliquescent salts of the magnesium chloride group, or of the calcium chloride group, have been found very satisfactory.

The steam introduced during the kneading or mixing operation diffuses the deliquescent salt through the mass or mix and the briquettes subsequently formed or molded therefrom have the salt or other deliquescent material distributed therethrough. This process has been found to be very satisfactory when either asphalt or coal tar pitch binders have been used, and even when a secondary binder is employed, such as sulphite liquor, starch or bentonite.

If desired, the deliquescent salt may be introduced in solution in the presence of this binding material, although when a solution is directly introduced into the mixture, the content of calcium chloride should be very high. For this purpose preferably a solution of a percentage as high as fifty percent (50%) calcium or magnesium chloride, or both, is used, for the reason that the moisture content of the solution lessens the adhesive effect of the binder. When the deliquescent salt is introduced before the briquette is molded, it is preferable to utilize the material in dry form, particularly if steam or other agents which

will diffuse the material through the mass are employed during the kneading operation.

After the briquette has been formed, or as it is formed, a deliquescent material may be applied to its surface, for instance, by maintaining moist or saturated with the solution, the forming rolls or molds of the apparatus. Such a method has been found useful either in lieu of, or in addition to, the introduction of dry deliquescent material in the mixture. This procedure thoroughly impregnates the surfaces of the briquettes, and it is found there is a penetration for a sufficient depth, thereby rendering the exterior of the briquette hygroscopic.

I have observed that this method, when employed for the application of deliquescent salts, affords good protection and improves the surfaces of the briquettes not only by allaying dust, but also by slowing down combustion. This slowing of combustion is probably due to an increased moisture content; it renders necessary higher temperatures before there can evolve the smoke-producing volatile gases contained in the binder.

As to the percentage of deliquescent material to be included, these will necessarily vary, because of the different types of combustible carbonaceous materials employed, and also because of the different binders utilized in briquette manufacture. If the briquette includes either as a binder or for other purposes, a material which is chemically active relative to the deliquescent material or salt, then, of course, it is necessary to utilize an amount of the latter sufficient to leave in the completed briquette a free or available portion of the deliquescent material, i. e., a portion over and above that neutralized by the reactive element in the mix, in order to produce a hygroscopic action.

However, it is preferable to utilize the binder which is chemically inactive or inert relative to the deliquescent material and to guard against the inclusion of ingredients which react chemically with the deliquescent material, and thus counteract its hygroscopic action. A binder such as coal tar pitch or asphalt is of this nature.

With briquettes of this composition, i. e., those which include an inactive or inert binder and no other elements which chemically modify the deliquescent salt, one percent (1%) of calcium chloride, magnesium chloride, other deliquescent salt will suffice as a deliquescent material content, and will afford the desired hygroscopic action. This content may be obtained by introducing dry or crystal magnesium or calcium chloride into the mixture, or by surface impregnation of the formed briquette. Or both modes of application may be adopted.

This amount of calcium chloride (1%) will not affect objectionably the adhesive action of the binder, although when a binder such as

sulphite liquor, which has an affinity for moisture and is itself hygroscopic is employed, it will be found preferably to utilize the surface impregnation method.

5 The percentage of calcium chloride or magnesium chloride may be varied considerable. For example, it has been found that the more friable or carbonaceous materials require a greater percentage of deliquescent salt than 10 the harder coals, which are not so dusty. When the allaying of dust is the only consideration, and the surface impregnation method is followed, it will be satisfactory if about one-eight ( $\frac{1}{8}$ ) to 1 quarter percent of 15 the completed briquette is a deliquescent material; but where it is desired to slow combustion and reduce the evolution of smoke during burning, the content of deliquescent material should be higher, and then it is preferable that the deliquescent material should 20 be introduced into the body of the briquette by other means than surface impregnation, either in addition to the surface impregnation or in lieu thereof. It has been found 25 that for improving the combustion and reducing smoke given off, the content of deliquescent materials of the nature of calcium chloride and magnesium chloride should be in the neighborhood of one percent (1%).

30 The following will serve as suitable examples of compositions which have been found satisfactory:

|                                                                                                                                                                                                                                                                            | 1  | Per cent |
|----------------------------------------------------------------------------------------------------------------------------------------------------------------------------------------------------------------------------------------------------------------------------|----|----------|
| 35 Coal                                                                                                                                                                                                                                                                    | 93 |          |
| Asphalt                                                                                                                                                                                                                                                                    | 6  |          |
| Calcium or magnesium chloride                                                                                                                                                                                                                                              | 1  |          |
|                                                                                                                                                                                                                                                                            | 2  |          |
| 40 Coal                                                                                                                                                                                                                                                                    | 92 |          |
| Asphalt                                                                                                                                                                                                                                                                    | 4  |          |
| Sulphite liquor                                                                                                                                                                                                                                                            | 3  |          |
| Calcium or magnesium chloride                                                                                                                                                                                                                                              | 1  |          |
|                                                                                                                                                                                                                                                                            | 3  |          |
| 45 Coal                                                                                                                                                                                                                                                                    | 93 |          |
| Asphalt                                                                                                                                                                                                                                                                    | 5  |          |
| Bentonite                                                                                                                                                                                                                                                                  | 1  |          |
| Calcium or magnesium chloride                                                                                                                                                                                                                                              | 1  |          |
|                                                                                                                                                                                                                                                                            | 4  |          |
| 50 Coal                                                                                                                                                                                                                                                                    | 93 |          |
| Coal tar pitch                                                                                                                                                                                                                                                             | 6  |          |
| Calcium or magnesium chloride                                                                                                                                                                                                                                              | 1  |          |
|                                                                                                                                                                                                                                                                            | 5  |          |
| 55 Coal                                                                                                                                                                                                                                                                    | 93 |          |
| Coal tar pitch                                                                                                                                                                                                                                                             | 5  |          |
| Bentonite                                                                                                                                                                                                                                                                  | 1  |          |
| Calcium or magnesium chloride                                                                                                                                                                                                                                              | 1  |          |
|                                                                                                                                                                                                                                                                            |    |          |
| 60                                                                                                                                                                                                                                                                         |    |          |
| In the above compositions the deliquescent salt has been included in dry form, and in lieu thereof by surface impregnation. Also both methods of introducing the deliquescent material have been utilized. That is to say, 65 a portion of the salt has been introduced in |    |          |

dry form and the remainder by impregnating the surface of the formed briquette by an aqueous solution.

It will be understood that both magnesium and calcium chloride may be used at the same time, if desired. The invention is characterized by the use of a coal which has not been treated with hygroscopic material, and from which, on the contrary, the moisture has been removed by drying and heating. Moreover, 70 the invention contemplates the mixing of the coal or other carbonaceous mass with the binder before the deliquescent material is introduced, so that the carbonaceous material may be subjected to the binder and coated 75 therewith before it is subjected to moisture resulting from the hygroscopic material.

The coal particles are thus treated thoroughly with the binder, and since they are free from moisture, the binder may cause adhesion of the various particles, more effectively than if the moisture content of the coal were high, or artificially raised by applying the deliquescent material thereto before the subjection of the coal to the binder. 80

In all of the various methods utilized there should be free or available material in the formed briquette. In some processes which involve the baking or coking of the molded briquette, it may be found desirable to impregnate the surface with the deliquescent material in solution after the coking operation. 95

Obviously, the invention is not limited to the details above set forth, and such variations may be made therein as come within the scope of the following claims which define the more essential features. 100

I claim:

1. The method of preparing fuel briquettes which comprises preliminarily drying a carbonaceous material, mixing therewith a binder, adding thereto a deliquescent salt in dry form and in sufficient quantity to be hygroscopically active, and molding the mixture. 105

2. The method of preparing fuel briquettes which comprises preliminarily drying a carbonaceous material, mixing therewith a binder, adding thereto a deliquescent salt in dry form and in sufficient quantity to be hygroscopically active, kneading the mixture, diffusing the salt through the mass by means of steam and then molding the briquette. 110

3. The method of preparing fuel briquettes which comprises preliminarily drying a carbonaceous material in finely divided form, mixing the finely divided carbonaceous material with a binder, adding thereto a deliquescent salt in dry form and in sufficient quantity to be free, whereby to exert a hygroscopic action, kneading the mixture, diffusing the salt by means of steam throughout the mass, molding the briquette and applying 115

125

130

plying a deliquescent salt in solution to the surface of the molded briquette.

4. The process of preparing fuel briquettes which comprises preliminarily drying a carbonaceous material in finely divided form, mixing the finely divided carbonaceous material, a deliquescent salt and a binder substantially chemically inactive relative to the material, whereby the latter may be hygroscopically active, molding the briquettes and applying a deliquescent salt in solution to the surface of the molded briquette.

5. A fuel briquette comprising finely divided substantially dry combustible carbonaceous material, a binder, and a deliquescent salt in dry form in sufficient quantity to be hygroscopically active.

6. A briquette comprising carbonaceous material, a binder, and a deliquescent salt coating the surface of the briquette and penetrating the briquette and extending below the surface thereof, said deliquescent salt being present in sufficient quantity to be hygroscopically active.

In testimony whereof I have hereunto set my hand.

GUSTAV KOMAREK.

30

35

40

45

50

55

60

65